

## UNITED STATES PATENT OFFICE

2,089,579

## TREATMENT OF HYDROCARBON OILS

Walter A. Schulze, Bartlesville, Okla., assignor to  
 Phillips Petroleum Company, Bartlesville,  
 Okla., a corporation of Delaware

No Drawing. Application September 10, 1934,  
 Serial No. 743,492

10 Claims. (Cl. 44-9)

This invention relates to the prevention of corrosion of metals, and refers more particularly to a new and improved treatment of hydrocarbon oils containing sulfur. It includes both the method of treatment and the product obtained.

More specifically this invention relates to the treatment of hydrocarbon liquid fuels ranging from liquefied petroleum gases through kerosene to prevent or retard or inhibit the corrosive action of elementary sulfur on such metals as copper, bronze, etc.

Gasolines as commercially produced always contain more or less elementary sulfur resulting from the oxidation or decomposition of hydrogen sulfide and/or organic sulfur compounds during fractionation or other heat treatment of these products. Furthermore, during the doctor sweetening operation wherein free sulfur is added to the oil for the purpose of converting the lead mercaptides to lead sulfide and alkyl disulfides, some excess of free sulphur must be used in order that the "breaking out" operation can be obtained in a reasonable amount of time. Therefore, regardless of how the oils are produced some free sulphur is practically certain to be present and such sulfur reacts readily with copper and its alloys when the said oils are in contact with such metals.

Similar problems or disadvantages are met with liquefied petroleum gases which is the name applied to a material similar to gasoline in physical properties but which consists largely of low boiling hydrocarbons such as propane and butane kept in the liquid state by the use of pressure. If such liquefied gases are drawn off in the vapor form then free sulphur will be concentrated in the containers and over a period of time the quantity may become quite large. It is common practice in dispensing liquefied petroleum gases to use certain materials containing copper and its alloys, and such materials are particularly subject to corrosion by free sulphur. This corrosion and consequent weakening of the materials is especially dangerous where such elevated pressures are necessary.

At the present time it is necessary to treat the crude hydrocarbon products by very rigorous and expensive methods in order that the quantity of free sulphur present in the finished products is sufficiently low that the rate of corrosion will not be exorbitant.

I have now discovered that by the addition of small amounts of certain compounds to the free sulphur containing hydrocarbon oils the corrosive action of the sulphur on such metals as

copper and its alloys is prevented or retarded or inhibited. The compounds which I include in this invention are those containing a hydroxyl and a carbonyl radical attached either to the same carbon atom or to its equivalent in a conjugated system. Polyhydroxy compounds and compounds containing nitrogen, e. g. the amino derivatives, are not intended to be included in this definition.



15

wherein the carbonyl group and the hydroxyl group are attached to the 1,4 carbons respectively of a conjugated system, is particularly outstanding in its effectiveness in preventing the action of free sulphur on copper. Other compounds of similar structure are fluorescein and phenolphthalein.



25

is an example of a compound wherein the carbonyl group and the hydroxyl group attached to the same carbon atom have given good results in preventing sulphur corrosion. The lactic acid esters, e. g. ethyl and butyl, are examples of other compounds belonging in this classification which have been found to be quite effective.

30

According to this invention a small amount of one of the compounds mentioned, e. g. para-hydroxy benzophenone, is added to a hydrocarbon oil containing elementary sulphur. In general the preferred actual concentration of the compound may vary between the limits of 0.001 percent to 0.1 percent. Such quantities give good 35 results but larger or smaller amounts of the inhibitor may be used without departing from the scope of this invention.

35

The amount of the compound needed to prevent corrosion of the copper depends to some extent on the amount of free sulphur in the hydrocarbon solution. The percent of the compound to be used in the oil depends, also, on the ratio of the surface area of the copper to the volume of the oil.

40

50

50

It is to be understood that the "corrosion-preventing" agent may be added either to a hydrocarbon oil already containing free sulfur or to an oil which may subsequently contain elementary sulfur as a result of the decomposition and/or

55

the oxidation of unstable sulfur compounds therein.

I have found that the various compounds are not equally effective and that much larger quantities of certain of the compounds must be used if equivalent effectiveness is to be obtained. In general the results indicate that (1) those compounds mentioned above containing the hydroxyl attached to the para position in the benzene nucleus with the general formula



15 wherein R represents either an alkyl or an aryl group are more effective than the aliphatic compounds mentioned above and (2) the simple alkyl groups such as methyl and ethyl are considerably better than butyl and amyl. It is believed that the molecules containing the longer chains are less tightly held (absorbed) on the surface of the copper and are thereby less effective than the molecules with the shorter chains.

20 25 One of the tests used for evaluating the effectiveness of these compounds is the corrosion test wherein a clean copper strip is immersed in the hydrocarbon oil and then heated at 140° F. for several hours. The duration of the heating period before appearance of discoloration on the copper strip is the measure of the corrosiveness of the oil. Another test which is used is that of merely noting the time during which no discoloration appears on the copper strip immersed 30 in a sulfur-bearing naphtha solution at room temperature.

35 The following examples will illustrate the usefulness of my process:

Example 1.—0.00086 percent elementary sulfur was added to a freshly distilled light naphtha. A copper strip immersed in a 60 cc. portion of this naphtha was quite badly corroded after standing 20 minutes at room temperature whereas a copper strip immersed in a similar portion of 40 the naphtha to which was added 0.005 percent para-hydroxy-benzophenone showed no discoloration or corrosion at the end of 71 days.

Example 2.—The copper strip immersed in a 50 cc. portion of naphtha containing 0.00086 45 percent elementary sulfur and a little para-hydroxy-benzophenone showed no discoloration after standing 6 hours at room temperature and heating three hours at 140° F. whereas the copper strip in the untreated sample was badly corroded in a short time at room temperature.

Example 3.—The copper strip immersed in a 50 cc. portion of naphtha containing 0.00086 55 percent elementary sulfur and a little n-butyl-d-l-malate showed no discoloration or corrosion after standing 6 hours at room temperature, 4 hours at 140° F. and 15 hours more at room temperature whereas the copper strip in the untreated sample was badly corroded within a few minutes at room temperature.

60 65 In a similar test n-butyl lactate was found to be quite effective at room temperature but somewhat less effective than the corresponding malate at elevated temperatures.

It is not desired to limit the invention to any 70 specific concentration of the treating agents since use may be made of higher or lower concentrations of any members of the classes of compounds mentioned herein and as a result thereof longer or shorter periods of preventing, 75 retarding or inhibiting corrosion of copper and

its alloys by elementary sulfur secured depending upon the specific agent used, the concentration of the agent, the percentage of free sulfur in the material treated and the conditions under which the subsequent storage takes place.

Obviously these various compounds differ greatly in their solubility in hydrocarbon oils. Some of them are practically insoluble while others are readily soluble. Inasmuch as the desired solubility can usually be obtained by 10 the introduction of "more oil soluble" or "less oil soluble" groups into such compounds, it is to be understood that such may be made without departing from the spirit and scope of this invention. Miscibility agents such as butyl alcohol can sometimes be added with the more insoluble compounds to increase their solubility in the hydrocarbon oils.

15 I claim:

20 25 1. The method of inhibiting the corrosion of copper and its alloys by hydrocarbon liquid fuels ranging from liquefied petroleum gases through kerosene, said liquid fuels containing sufficient elementary sulfur so that they tend normally to corrode copper and its alloys, which comprises adding to the said liquid fuels a small amount of a compound of the structure



30 wherein R represents a member selected from the group consisting of the alkyl and aryl groups.

35 40 45 50 55 60 65 70 75 80 85 90 95 2. The method of inhibiting the corrosion of copper and its alloys by hydrocarbon liquid fuels ranging from liquefied petroleum gases through kerosene, said liquid fuels containing sufficient elementary sulfur so that they tend normally to corrode copper and its alloys, which comprises adding to the said liquid fuels a small amount of para-hydroxy-benzophenone.

3. Predominantly hydrocarbon liquid fuels ranging from liquefied petroleum gases through kerosene containing sufficient elementary sulfur to tend normally to corrode copper and its alloys to which has been added as a corrosion inhibitor a small amount of a compound of the structure



50 55 60 65 70 75 80 85 90 95 wherein R represents a member selected from the group consisting of the alkyl and aryl groups.

4. Predominantly hydrocarbon liquid fuels ranging from liquefied petroleum gases through kerosene containing sufficient elementary sulfur to tend normally to corrode copper and its alloys to which has been added as a corrosion inhibitor a small amount of para-hydroxy-benzophenone.

5. Motor fuel containing sufficient elementary sulfur to tend normally to corrode copper and its alloys in contact with said fuel, to which has been added as a corrosion inhibitor a small amount of a compound of the structure



60 65 70 75 80 85 90 95 wherein R represents a member selected from the group consisting of the alkyl and aryl groups.

6. Motor fuel containing sufficient elementary sulfur to tend normally to corrode copper and its alloys in contact with said fuel, to which has been added as a corrosion inhibitor a small amount of para-hydroxy-benzophenone.

7. The method of inhibiting the corrosion of copper and its alloys by light hydrocarbon oils substantially free of unsaturated hydrocarbons but containing sufficient elementary sulfur to tend normally to corrode copper and its alloys, which comprises adding to the said liquid fuels a small amount of a compound of the structure



wherein R represents a member selected from the group consisting of the alkyl and aryl groups.

8. Light hydrocarbon oil substantially free of unsaturated hydrocarbons containing sufficient sulfur so that they tend normally to corrode copper and its alloys to which has been added as a corrosion inhibitor a small amount of para-hydroxy-benzophenone.

9. Liquefied petroleum gas containing sufficient elementary sulfur to tend normally to corrode copper and its alloys in contact with said fuel, to which has been added as a corrosion inhibitor a small amount of a compound of the structure 5



wherein R represents a member selected from the 10 group consisting of the alkyl and aryl groups.

10. Liquefied petroleum gas containing sufficient elementary sulfur to tend normally to corrode copper and its alloys in contact with said fuel to which has been added as a corrosion 15 inhibitor a small amount of para-hydroxy-benzophenone.

WALTER A. SCHULZE.